# EUROPEAN PATENT SPECIFICATION

(11) **EP 3 214 191 B1**
(45) Date of publication and mention of the grant of the patent: **19.08.2020**
(21) Application number: 17468001.7
(22) Date of filing: 02.03.2017
(51) Int. Cl.: C22C 21/02, C22F 1/05

(54) **A HIGH-STRENGTH AL-MG-SI ALUMINIUM ALLOY AND ITS MANUFACTURING PROCESS**
HOCHFESTE AL-MG-SI-ALUMINIUMLEGIERUNG UND DEREN HERSTELLUNGSVERFAHREN
ALLIAGE D'ALUMINIUM AL-MG-SI À HAUTE RÉSISTANCE ET SON PROCÉDÉ DE FABRICATION

(30) Priority: 04.03.2016 SI 201600063
(43) Date of publication of application: 06.09.2017
(73) Proprietor: Impol 2000, d. d., 2310 Slovenska Bistrica (SI)
(72) Inventor: Cvahte, Peter, 2310 Slovenska Bistrica (SI); Jelen, Marina, 2310 Slovenska Bistrica (SI); Vukasin, Dragojevic, 2314 Zgornja Polskava (SI); Matej, Steinacher, 2317 Oplotnica (SI)

(56) References cited:
- EP-A1- 2 799 564
- EP-A1- 2 883 973

## Description

The invention is in the field of metallurgy and materials and refers to a high-strength Al-Mg-Si aluminium alloy and its manufacturing process. The invented alloy is used in the automotive, aircraft, transport, and construction industries.

Trends in the modern vehicle-producing industry include the manufacturing of so-called green transportation vehicles. These vehicles have lower fuel consumptions and CO₂ emissions through a reduction in their weight. However, the user's safety must also be considered. In practice this means that the heavy steel parts must be exchanged for lighter materials, such as high-strength Al-Mg-Si aluminium alloys (the 6xxx series).

Magnesium and silicon are the main alloying elements in the 6xxx aluminium alloys. Together they form the Mg₂Si phase, which allows precipitation hardening of the alloy during ageing. The Al-Mg-Si alloys have good workability, machinability, weldability, corrosion resistance, and strength between 230 and 450 MPa, depending on the heat treatment. A strength above 450 MPa was achieved with addition of 0.8-1.5 wt. % of Cu and 0.05-0.3 wt. % of Zr in the EP 2548983 patent, but this alloy has poor corrosion resistance on account of the higher content of copper. On the other hand, the Al-Zn alloys (the 7xxx series) can achieve a strength higher than 500 MPa, but the use of these alloys is limited by their workability and corrosion resistance.

The Al-Mg-Si alloys are manufactured in the following sequence: charge preparing and melting, melt holding, semi-continuous billet casting, homogenizing, extruding of the bars or other final forms, forming (e.g. forging), and heat treatment. A recent manufacturing process, i.e., the continuous casting of bars, enables the forming of cast bars directly. In this case there is no homogenizing and extrusion.

Besides magnesium and silicon, the Al-Mg-Si alloys contain iron, copper, manganese, chromium, zinc, titanium, and zirconium. The addition of zirconium improves the corrosion resistance, inhibits the recrystallization, refines the as-cast grains, and consequently improves the mechanical properties. The content of zirconium in the Al-Mg-Si alloys is to 0.3 wt. % [EP 1458898, EP 2554698, EP 2799564, EP 2644725, EP 2811042, EP 2003219, EP 0987344, EP 1737994, EP 0173632, EP 0787217, EP 1802782, JP 2004043907, JP 2001107168, JP 2003277868, US 2004062946, JP 2007177308, US 2010089503, US 5240519]. The process parameters also depend on the content of zirconium in Al-Mg-Si alloys.

Until now the chemical compositions of Al-Mg-Si alloys do not contain 1.3-1.7 wt. % of Si, 0.14-0.25 wt. % of Fe, up to 0.75 wt. % of Cu, 0.7-0.8 wt. % of Mn, 0.85-1.1 wt. % of Mg, 0.15-0.25 wt. % of Cr, up to 0.2 wt. % of Zn, up to 0.1 wt. % of Ti, 0.15-0.25 wt. % of Zr, other elements up to 0.15 wt. % (single element up to 0.05 wt. %), with the rest being Al. The present invention is defined by the appended claims.

The content and effect of each element in the invented Al-Mg-Si alloy are described below:
- Silicon (Si: 1.3 to 1.7 wt. %) is one of the major elements of the alloy in the present invention, along with Mg and Cu, which improves the strength. Si is combined with Mg and forms Mg₂Si, which precipitation hardens the α-Al matrix during the artificial ageing. Although the contribution of the precipitation hardening is increased when the content of Si exceeds 1.7 wt. %, the stress-corrosion cracking resistance and the corrosion resistance are aggravated. Also, coarse β-Si particles are precipitated, which likewise deteriorates the corrosion resistance and toughness. The contribution of the precipitation hardening is decreased when the content of Si is less than 1.3 wt. %.
- Iron (Fe: 0.14 to 0.25 wt. %) forms Al-Fe-Si-(Mn, Cr) phases and Al₇Cu₂Fe, Al₁₂(Fe, Mn)₃Cu₂, or Al₆(Fe, Mn) precipitates. The fractions of these phases and precipitates increase when the content of Fe exceeds 0.25 wt. %, and this deteriorates the mechanical properties, corrosion resistance, and machinability.
- Copper (Cu: to 0.75 wt. %) is one of the elements, along with Si and Mg, which improve the strength of the alloy with precipitation hardening of the α-Al matrix during the artificial ageing. The effect of the precipitation hardening is increased in proportion with the content of Cu. When it exceeds 0.75 wt. %, the sensitivity to stress corrosion cracking and intergranular corrosion is increased, which reduces the durability of the aluminium alloy.
- Manganese (Mn: 0.7 to 0.8 wt. %) forms, together with Fe, Si, and Cr, the AI-Fe-Si-(Mn, Cr) phase and Al₆Mn dispersed particles, which are formed during the homogenization and solution heat treatment. These dispersed particles also inhibit the grain growth. The fine crystal grains and sub grains improve the mechanical properties, fracture toughness, and fatigue properties. With a content of Mn under 0.7 wt. % the alloy is liable to recrystallize. On the other hand, when the content of Mn exceeds 0.8 wt. %, the coarse Al₆Mn dispersed particles are formed and deteriorate both the mechanical properties and the formability.
- Magnesium (Mg: 0.85-1.1 wt. %) in combination with Si forms the Mg₂Si phase at the grain boundaries during the solidification. The Mg₂Si phase is partially dissolved in the α-Al matrix during the homogenization and the remainder stays at the grain boundaries. The undissolved Mg₂Si particles inhibit the grain growth during subsequent processes. The dissolved Mg and Si are precipitated as Mg₂Si during the artificial ageing, which then hardens the α-Al matrix. The precipitation hardening is reduced when the content of Mg is below 0.85 wt. % and increased when the content of Mg exceeds 1.1 wt. %, but the coarse Mg₂Si precipitates decrease the elongation, deteriorate the forgeability and lower the intergranular corrosion resistance.
- Chromium (Cr: 0.15 to 0.25 wt. %) along with Fe, Si, and Mn forms the Al-Fe-Si-(Mn, Cr) phase during solidification and forms Si₁₂Mg₂Cr and Al₂Mg₂Cr dispersed precipitates during the homogenization. These precipitates inhibit the grain growth. The coarse AI-Fe-Si-(Mn, Cr) phases are formed above 0.25 wt. % of Cr and represent the initial sites for crack formation.
- Zinc (Zn: to 0.2 wt. %) and Mg form MgZn₂ precipitates during the precipitation hardening, which contribute to the strength of the aluminium alloy. On the other hand, when MgZn₂ is precipitated, the content of Mg in the alloy is decreased. This leads to a decreasing fraction of Mg₂Si precipitates, which contribute more to the strength than the MgZn₂ precipitates. The Zn also deteriorates the corrosion resistance.
- Titanium (Ti: to 0.1 wt. %) is added to aluminium alloys with an Al-Ti-B master alloy, where it is precipitated in the form of Al₃Ti and TiB₂ particles. The Al₃Ti particles are dissolved faster in the melt, while the TiB₂ particles coated with a thin Al₃Ti layer act as efficient nuclei for the grain growth of the as-cast α-Al grains. The Ti that is dissolved in the melt also inhibits the grain growth of the α-Al. The fine-grained microstructure improves the workability and mechanical properties of the alloy.
- Zirconium (Zr: 0.15 to 0.25 wt. %) forms fine Al₃Zr and Si₂Zr precipitates at the grain boundaries and sub grains during the homogenization. The precipitates improve the corrosion resistance, inhibit the recrystallization, and consequently improve the mechanical properties.
- Other elements (to 0.15 wt. %; single element to 0.05 wt. %) are presented as trace elements and a small quantity of these elements do not effect to the properties of the aluminium alloy.

The manufacturing process of the Al-Mg-Si alloy (Figure 1) begins with preparing a charge that consists of the primary aluminium (99.7 wt. % of Al), revert scrap, secondary scrap, and alloying elements. These are added as the pure elements or master alloys. The prepared charge is placed in the melting furnace (gas or induction), where the melting is started. The chemical composition of the melt is checked after the melting. The melting temperature depends on the content of Zr in the melt and is between 700 and 780 °C, while the melting takes up to 5 h. The melt stirring is favourable for the dissolution of Zr, which is implemented naturally in an induction furnace and mechanically in a gas furnace. The melting time is reduced with the use of an Al-Zr master alloy, where the Zr is precipitated in the form of fine Al₃Zr phases. When the chemical composition is achieved, the melt is poured into the holding furnace, where it is cleaned with argon or nitrogen flushing and is held above the liquidus temperature up to 4 h. The liquidus temperature depends on the content of Zr in the melt and is between 700 and 750 °C. If the holding temperature falls below the liquidus temperature, the zirconium begins to precipitate in the form of the Al₃Zr phase, which settles to the bottom of the holding furnace, because its density is 4.1 g/cm³. The coarse Al₃Zr phases represent the defects in the final products and also decrease the effect of the Zr in the alloy. In the first case, the alloy can be semi-continuously cast with different casting processes (with floats, with a hot top, or in an electromagnetic field at lower frequency) into billets with a diameter of 218-450 mm and a length up to 8 m. The casting temperature is between 680 and 730 °C and the casting rate is 50-85 mm/min. In the second case, the alloy can be continuously cast into bars with a diameter of 30-150 mm. The casting temperature is between 680 and 730 °C and the casting rate is 100-1000 mm/min. The cast bars are subsequently hot or cold formed and heat treated, or only heat treated. The melt temperature in the holding furnace should not fall under the liquidus temperature during the casting. The cast billets are homogenized at a temperature of 400-550 °C for up to 24 h, cooled with fans, water fog, water, or air, and ultrasonically tested. The homogenization is performed below the solidus temperature, because the Mg₂Si phases are melted at higher temperatures and cause the formation of pores within the microstructure. Then the billets are cut into a round length of 600-1600 mm and dressed as necessary. Later, the round is preheated to the homogenous temperature or in the temperature profile (wedge). The temperature of the round is between 470 and 550 °C. The bars, with a diameter of 20-180 mm or other forms to an outlined circle of 270 mm, are directly or indirectly extruded with an extrusion rate of 0.1-25 mm/s. The temperatures of the container and the die are between 360 and 520 °C. The bars are water quenched (spray or wave) immediately after the extrusion (T1 temper). Then the bars in the T1 temper are cold or hot formed and heat treated, or only heat treated according to the required heat treatment. The bars, other forms, or forged parts for the T6 temper are solution heat treated at a temperature of 450-550 °C from 1 to 3 h, water quenched, and artificially aged at a temperature of 120-210 °C for up to 15 h. For the T5 temper they are only artificially aged at a temperature of 120-210 °C for up to 15 h and for the T4 temper they are the solution heat treated at a temperature of 450-550 °C from 1 to 3 h, water quenched, and still naturally aged.

The high-strength Al-Mg-Si aluminium alloy, in the form of bars, other forms, or forged parts, which is manufactured with the processes and chemical composition described above, achieves a tensile strength of 452-495 MPa, a yield stress of 418-465 MPa, an elongation of 9-12.5 %, and a hardness of 141-145 HB in the T6 temper. Besides the high mechanical properties, the alloy has good corrosion resistance, which is in accordance with automotive standards. The intergranular corrosion test according to the VW PV 1113 standard showed that the depth of the intergranular corrosion of the bars in the T6 temper is less than 200 µm.

## Claims

1. A high-strength extruded or cast Al-Mg-Si aluminium alloy **characterized in,**
**that** it contains 1.3-1.7 wt. % of Si, 0.14-0.25 wt. % of Fe, up to 0.75 wt. % of Cu, 0.7-0.8 wt. % of Mn, 0.85-1.1 wt. % of Mg, 0.15-0.25 wt. % of Cr, up to 0.2 wt. % of Zn, up to 0.1 wt. % of Ti, 0.15-0.25 wt. % of Zr, and other elements up to 0.15 wt. %, single element to 0.05 wt. %, and the rest being Al.

2. A manufacturing process of the high-strength extruded or cast Al-Mg-Si aluminium alloy with composition according to claim 1, **characterized in,**
**that** it includes the charge preparing, melting, melt holding, semi-continuous billet casting or continuous bar casting, homogenizing, cutting of the billets, extruding, forming, and heat treatment.

3. The process according to the claim 2 is **characterized in,**
**that** the melt temperature in the melting furnace is from 700 to 780 °C and the melting time up to 5 h.

4. The process according to the claim 2 is **characterized in,**
**that** the melt temperature in the holding furnace is from 700 to 750 °C and the holding time before the casting is up to 4 h, while the melt temperature in the holding furnace should not fall below the liquidus temperature during casting.

5. The process according to the claim 2 is **characterized in,**
**that** the casting is implemented with a semi-continuous casting process with floats, with a hot top, or in an electromagnetic field at lower frequency into billets with a diameter of 218-450 mm, length up to 8 m, at a casting temperature of 680-730 °C, and a casting rate of 50-85 mm/min or that the casting is implemented with a continuous casting process into bars with a diameter of 30-150 mm, at a casting temperature of 680-730 °C, and at a casting rate of 100-1000 mm/min.

6. The process according to the claim 2 is **characterized in,**
**that** the cast billets are homogenized at a temperature of 400-550 °C for up to 24 h and cooled with fans, water fog, water, or air.

7. The process according to the claim 2 is **characterized in,**
**that** the rounds are preheated to a temperature of 470-550 °C before the extrusion.

8. The process according to the claim 2 is **characterized in,**
**that** the container temperature and the die temperature are between 360 and 520 °C for a direct or indirect extrusion.

9. The process according to the claim 2 is **characterized in,**
**that** the rounds are directly or indirectly extruded into bars with a diameter of 20-180 mm or other forms to an outlined circle of 270 mm with an extrusion rate of 0.1-25 mm/s, which are still water quenched (spray or wave) immediately after the extrusion.

10. The process according to the claim 2 is **characterized in,**
**that** the bars, other forms, or forged parts for the T6 temper are solution heat treated at a temperature of 450-550 °C from 1 to 3 h, water quenched, and artificially aged at a temperature of 120-210 °C for up to 15 h.

11. The process according to the claim 2 is **characterized in,**
**that** the bars, other forms, or forged parts for the T5 temper are artificially aged at a temperature of 120-210 °C for up to 15 h.

12. The process according to the claim 2 is **characterized in,**
**that** the bars, other forms, or forged parts for the T4 temper are solution heat treated at a temperature of 450-550 °C from 1 to 3 h, water quenched, and then naturally aged.

## Patentansprüche

1. Eine hochfeste gespritzte oder gegossene Al-Mg-Si-Aluminiumlegierung ist **dadurch gekennzeichnet,**
**dass** sie 1,3-1,7 Gew.-% Silicium (Si), 0,14-0,25 Gew.-% Eisen (Fe), bis zu 0,75 Gew.-% Kupfer (Cu), 0,7-0,8 Gew.-% Mangan (Mn), 0,85-1,1 Gew.-% Magnesium (Mg), 0,15-0,25 Gew.-% Chrom (Cr), bis zu 0,2 Gew.-% Zink (Zn), bis zu 0,1 Gew.-% Titan (Ti), 0,15-0,25 Gew.-% Zirconium (Zr), sowie andere Elemente bis zu 0,15 Gew.-% und ein Einzelelement bis 0,05 Gew.-% enthält, und der Rest aus Aluminium (AI) besteht.

2. Ein Herstellungsprozess der hochfesten gespritzten oder gegossenen Al-Mg-Si-Aluminiumlegierung mit einer Zusammensetzung gemäß Anspruch 1, ist **dadurch gekennzeichnet,**
**dass** er die Vorbereitung des Auftrags, das Schmelzen, die Schmelzwarmhaltung, den semi-kontinuierlichen Rundbarrenguss oder den kontinuierlichen Balkenguss, das Homogenisieren, das Schneiden der Rundbarren, das Spritzen, Formen und die Wärmbehandlung beinhaltet.

3. Das Verfahren gemäß Anspruch 2 ist **dadurch gekennzeichnet,**
**dass** die Schmelztemperatur im Schmelzofen zwischen 700 und 780 °C liegt und dass die Schmelzzeit bis zu 5 Stunden beträgt.

4. Das Verfahren gemäß Anspruch 2 ist **dadurch gekennzeichnet,**
**dass** die Schmelztemperatur im Warmhalteofen zwischen 700 und 750 °C liegt und dass die Warmhaltezeit vor dem Gießen bis zu 4 Stunden dauert, während die Schmelztemperatur im Warmhalteofen während des Gießens nicht unter die Liquidustemperatur sinken sollte.

5. Das Verfahren gemäß Anspruch 2 ist **dadurch gekennzeichnet,**
**dass** der Guss mit einem halb-kontinuierlichen Gießverfahren mit Schwimmern, mit Gießaufsatz oder in einem elektromagnetischen Feld bei niedrigerer Frequenz zu Rundbarren mit einem Durchmesser von 218-450 mm, einer Länge bis zu 8 m, bei einer Gießtemperatur von 680-730 °C und einer Gießgeschwindigkeit von 50-85 mm/min durchgeführt wird, oder dass der Guss mit einem kontinuierlichen Gießverfahren zu Barren mit einem Durchmesser von 30-150 mm, bei einer Gießtemperatur von 680-730 °C und einer Gießgeschwindigkeit von 100-1000 mm/min durchgeführt wird.

6. Das Verfahren gemäß Anspruch 2 ist **dadurch gekennzeichnet,**
**dass** die gegossenen Rundbarren bei einer Temperatur von 400-550 °C bis zu 24 Stunden homogenisiert werden und mit Gebläsen, Wassernebel, Wasser oder Luft gekühlt werden.

7. Das Verfahren gemäß Anspruch 2 ist **dadurch gekennzeichnet,**
**dass** die Rundbarren vor dem Strangpressen auf eine Temperatur von 470-550 °C vorgeheizt werden.

8. Das Verfahren gemäß Anspruch 2 ist **dadurch gekennzeichnet,**
**dass** die Behältertemperatur und die Formtemperatur beim direkten oder indirekten Strangpressen zwischen 360 und 520 °C liegen.

9. Das Verfahren gemäß Anspruch 2 ist **dadurch gekennzeichnet,**
**dass** die Rundbarren direkt oder indirekt in Balken mit einem Durchmesser von 20-180 mm oder in andere Formen auf eine skizzierte Kreisform von 270 mm stranggepresst werden (und zwar mit einer Extrusionsgeschwindigkeit von 0,1-25 mm/s), die dennoch sofort nach dem Strangpressen wasservergütet werden (mittels Sprühwasser oder Welle).

10. Das Verfahren gemäß Anspruch 2 ist **dadurch gekennzeichnet,**
**dass** die Balken, sonstige Formen oder Schmiedeteile für den Härtegrad T6 bei einer Temperatur von 450-550 °C für 1 bis 3 Stunden lösungsgeglüht, wasservergütet und bei einer Temperatur von 120-210 °C für bis zu 15 Stunden warmausgehärtet werden.

11. Das Verfahren gemäß Anspruch 2 ist **dadurch gekennzeichnet,**
**dass** die Balken, sonstige Formen oder Schmiedeteile für den Härtegrad T5 bei einer Temperatur von 120-210°C für bis zu 15 Stunden warmausgehärtet werden.

12. Das Verfahren gemäß Anspruch 2 ist **dadurch gekennzeichnet,**
**dass** die Balken, sonstige Formen oder Schmiedeteile für den Härtegrad T4 bei einer Temperatur von 450-550 °C für 1 bis 3 Stunden lösungsgeglüht, wasservergütet und dann kaltausgehärtet werden.

## Revendications

1. Alliage d'aluminium extrudé ou coulé Al-Mg-Si à haute résistance mécanique, **qui se caractérise en ceci**
qu'il contient 1,3 à 1,7 % en poids de Si, 0,14 à 0,25 % en poids de Fe, jusqu'à 0,75 % en poids de Cu, 0,7 à 0,8 % en poids de Mn, 0,85 à 1,1 % en poids de Mg, 0,15 à 0,25 % en poids de Cr, jusqu'à 0,2 % en poids de Zn, jusqu'à 0,1 % en poids de Ti, 0,15 à 0,25 % en poids de Zr et d'autres éléments jusqu'à 0,15 % en poids, un seul élément jusqu'à 0,05 % en poids et le reste étant de l'Al.

2. Procédé de fabrication de l'alliage d'aluminium Al-Mg-Si extrudé ou coulé à haute résistance mécanique avec une composition selon la revendication 1, **qui se caractérise en ceci**
qu'il comprend la préparation de la charge, la fusion, le maintien en fusion, la coulée semi-continue en billettes ou en barres continues, l'homogénéisation, la coupe des billettes, l'extrusion, le formage et le traitement thermique.

3. Le procédé selon la revendication 2 se **caractérise par le fait**
**que** la température de fusion dans le four de fusion est de 700 à 780 °C et le temps de fusion peut atteindre 5 h.

4. Le procédé selon la revendication 2 se **caractérise par le fait**
**que** la température de fusion dans le four de maintien est de 700 et 750 °C et que le temps de maintien avant la coulée peut atteindre 4 h, tandis que la température de fusion dans le four de maintien ne doit pas être inférieure à la température du liquidus pendant la coulée.

5. Le procédé selon la revendication 2 se **caractérise par le fait**
**que** la coulée est réalisée par un procédé de coulée semi-continue avec des flotteurs, avec un dessus chaud ou dans un champ électromagnétique à basse fréquence dans des billettes d'un diamètre de 218 à 450 mm, d'une longueur pouvant atteindre 8 m, à une température de coulée de 680 à 730 °C et une vitesse de coulée de 50 à 85 mm/min ou que la coulée est réalisée par un procédé de coulée continue en barres d'un diamètre de 30 à 150 mm, à une température de coulée de 680 à 730°C et une vitesse de coulée de 100 à 1000 mm/min.

6. Le procédé selon la revendication 2 se **caractérise par le fait**
**que** les billettes coulées sont homogénéisées à une température de 400 à 550 °C pendant 24 h maximum et refroidies avec des ventilateurs, du brouillard d'eau, de l'eau ou de l'air.

7. Le procédé selon la revendication 2 se **caractérise par le fait**
**que** les ronds sont préchauffés à une température de 470 à 550 °C avant l'extrusion.

8. Le procédé selon la revendication 2 se **caractérise par le fait**
**que** la température du conteneur et à la matrice est comprise entre 360 et 520 °C pour une extrusion directe ou indirecte.

9. Le procédé selon la revendication 2 se **caractérise par le fait**
**que** les ronds sont extrudés directement ou indirectement en barres d'un diamètre de 20 à 180 mm ou d'autres formes en un cercle de 270 mm avec une vitesse d'extrusion de 0,1 à 25 mm/s, qui sont trempées à l'eau plate (pulvérisation ou vague) immédiatement après l'extrusion.

10. Le procédé selon la revendication 2 se **caractérise par le fait**
**que** les barres, autres formes ou pièces forgées pour la trempe T6 sont traitées thermiquement en solution à une température de 450 à 550 °C pendant 1 à 3 h, trempées à l'eau et vieillies artificiellement à une température de 120 à 210 °C pendant 15 h au maximum.

11. Le procédé selon la revendication 2 se **caractérise par le fait**
**que** les barres, autres formes ou pièces forgées pour la trempe T5 sont soumises à un vieillissement artificiel à une température de 120 à 210 °C pendant 15 heures au maximum.

12. Le procédé selon la revendication 2 se **caractérise par le fait**
**que** les barres, autres formes ou pièces forgées pour la trempe T4 sont traitées thermiquement en solution à une température de 450 à 550 °C pendant 1 à 3 h, trempées à l'eau, puis vieillies naturellement.
